# EUROPEAN PATENT SPECIFICATION

(11) **EP 0 586 943 B1**
(45) Date of publication and mention of the grant of the patent: **04.11.1998**
(21) Application number: 93113249.2
(22) Date of filing: 19.08.1993
(51) Int. Cl.: H01J 17/16, H01J 17/49

(54) **Process of making a plasma display apparatus**
Verfahren zur Herstellung eines Plasma-Anzeigegeräts
Procédé de fabrication d'un appareil d'affichage à plasma

(30) Priority: 21.08.1992 JP 222413/92
(43) Date of publication of application: 16.03.1994
(73) Proprietor: E.I. DU PONT DE NEMOURS AND COMPANY, Wilmington Delaware 19898 (US)
(72) Inventor: Borland, William, Cary, North Carolina 27513 (US); Kuwada, Ryosuke, Tokyo 206 (US); Nishi, Noboru, Tama-shi, Tokyo 206 (JP); Wang, Carl Baasun, Tokyo 152 (JP); Yamamoto, Yasuo, Fuchu-shi, Tokyo 183 (JP)
(74) Representative: von Kreisler, Alek, Dipl.-Chem.

(56) References cited:
- EP-A- 0 382 260
- WO-A-91/06118
- US-A- 5 037 723

## Description

### FIELD OF INVENTION

The invention relates to a process of making a plasma display apparatus comprising a plurality of stripe-shaped electrodes arranged in a matrix, a dot-shaped discharge area or pixel area at each solid intersection between said stripe-shaped electrodes and a fluorescent film formed on each of said discharge areas and adapted to emit light when said fluorescent film is excited by ultraviolet rays from the corresponding dischare area.

### BACKGROUND OF THE INVENTION

A plasma display apparatus typically comprises a pair of forward and backward insulation substrates arranged opposed to each other to form a discharge space therebetween, said discharge space containing a gaseous mixture of He with a trace of Xenon and others, a group of stripe-shaped electrodes on the opposed surfaces of said insulation substrates, said stripe-shaped electrodes being arranged to form a matrix pattern in said discharge space, said matrix parting said discharge space into a plurality of discharge gas containing sub-spaces, each intersection between said stripe-shaped electrodes corresponding to a pixel, and a fluorescent film in each of said sub-spaces.

More particularly, as shown in Fig. 10, the forward insulation substrate 1 is formed of sheet glass, with the internal surface thereof including a film-type light-blocking mask 2 formed thereon and first stripe-shaped electrodes 3 arranged side by side on the internal surface of the substrate 1 in one direction, these electrodes 3 functioning as anodes. The internal surface of the other or backward substrate 4 is similarly formed of sheet glass and the internal surface thereof includes second stripe-shaped electrodes 7 arranged to extend in a direction perpendicular to the lengths of the first electrodes 3, these electrodes 7 functioning as cathodes. The first and second electrodes 3, 7 are separated from each other by dielectric partitions 8. A dot-like discharge area 9 is formed at each of the intersections between the first and second electrodes 3, 7. The discharge area 9 contains a discharge gas containing Xenon. A dot-like fluorescent film 10 for color display is formed on the surface of each of the second electrodes 3.

Each of the partitions 8 is formed to have a thickness ranged between 100 µm and 200 µm by repeated thick-film printing of insulation paste. The discharge gas is a two-component mixture gas containing He and Xe, a three-component mixture gas containing He, Xe and any other suitable component or a single gas (e.g. Xe). The discharge gas is sealed within the corresponding discharge area 9 under the pressure of 1.3 to 66.7 kPa (10 to 500 Torr), depending on the composition thereof. Such a plasma display apparatus of the prior art (e.g. EP-A-0382260) was provided by repeating the thick film process to form partitions having a thickness ranged between 100 µm and 200 µm on an insulation substrate to define a plurality of dot-like discharge areas thereon or by performing the thick film printing process to form partitions as described, applying a paste containing silver in a groove surrounded and defined by said partitions, and firing the paste to form a group of electrodes. Thereafter, a fluorescent material is placed and fired in a recess formed by said partitions to form a fluorescent member covering one of the electrodes (i.e. one disposed on the backside of the substrate). When these frontside and backside substrates are superposed on each other, sealing, discharging and other gases are sealed therebetween to complete a plasma display apparatus.

The prior art process requires too many producing steps which would reduce the mass-producibility and increase the manufacturing cost. Since the electrodes, partitions and others are formed by repeating the thick-wall printing and firing steps, possible dot pitch is limited. The thickness of film must be controlled with high accuracy. Further, the substrates must be superposed and fixed to each other with a high precision. On the other hand, WO 91/06118 discloses a diffusion pattering process involving one patterned and one unpatterned dielectric.

### SUMMARY OF THE INVENTION

An object of the invention is to provide a process of making a plasma display apparatus, which process can more easily and effectively produce a plasma display apparatus having a number of electrodes disposed with a reduced dot pitch.

The invention is therefore directed to
(1) a process of making a plasma display apparatus, comprising the steps of providing dielectric substrates; forming a plurality of first electrodes on one of said substrates to extend in one direction; forming a plurality of second electrodes on the other substrate to extend in another direction perpendicular to said one direction; forming a ridge on at least one of said substrates to define a plurality of pixel areas; and providing fluorescent materials in said pixel areas, wherein the ridge is fabricated by a negative-acting diffusion patterning process comprising the sequential steps:
   a. Applying to at least one of the substrate an unpatterned first layer comprising a solid organic polymer which is soluble in a predetermined solvent or water;
   b. Applying to the unpatterned first layer a patterned second layer comprising a solubilizing agent which is capable of increasing the solubility of the organic polymer in the predetermined solvent or water;
   c. Heating the patterned second layer to effect patterned diffusion of the solubilizing agent into the underlying first organic polymer layer to render the diffusion patterned areas of the polymer in the first layer soluble in the predetermined solvent or water;
   d. Developing the underlying patterned layers by washing with predetermined solvent or water;
   e. Repeating a series of the above steps (a) to (d) to build thicker or more raised ridges; and
   f. Firing the patterned dielectric ridges;
(2) a process of making a plasma display apparatus, comprising the steps of providing dielectric substrates; forming a plurality of first electrodes on one of said substrates to extend in one direction; forming a plurality of second electrodes on the other substrate to extend in another direction perpendicular to said one direction; forming a ridge on at least one of said substrates to define a plurality of pixel areas; and providing fluorescent materials in said pixel areas, wherein the ridge is fabricated by a negative-acting diffusion patterning process comprising the sequential steps:
   a. Applying to at least one of the substrate an unpatterned first layer comprising a solid organic polymer which is soluble in a predetermined solvent or water;
   b. Applying to the unpatterned first layer a patterned second layer comprising a solubilizing agent which is capable of increasing the solubility of the organic polymer in the predetermined solvent or water;
   c. Heating the patterned second layer to effect patterned diffusion of the solubilizing agent into the underlying first organic polymer layer to render the diffusion patterned areas of the polymer in the first layer soluble in the predetermined solvent or water;
   d. Repeating the series of steps (a) to (c);
   e. Co-developing the underlying patterned layers by washing with predetermined solvent or water; and
   f. Firing the patterned dielectric ridges;
(3) a process of making a plasma display apparatus, comprising the steps of providing dielectric substrates; forming a plurality of first electrodes on one of said substrates to extend in one direction; forming a plurality of second electrodes on the other substrate to extend in another direction perpendicular to said one direction; forming a ridge on at least one of said substrates to define a plurality of pixel areas; and providing fluorescent materials in said pixel areas, wherein the ridge is fabricated by a positive-acting diffusion patterning process comprising the sequential steps:
   a. Applying to at least one of the substrate an unpatterned first layer comprising a solid organic polymer which is soluble in a predetermined solvent or water;
   b. Applying to the unpatterned first layer a patterned second layer comprising a desolubilizing agent which is capable of decreasing the solubility of the organic polymer in the predetermined solvent or water;
   c. Heating the patterned second layer to effect patterned diffusion of the desolubilizing agent into the underlying first organic polymer layer to render the diffusion patterned areas of the polymer in the first layer insoluble in the predetermined solvent or water;
   d. Developing the non-patterned areas of the underlying first layer by washing with predetermined solvent water;
   e. Repeating a series of the above steps (a) to (d) to build thicker or more raised ridges; and
   f. Firing the patterned dielectric ridges; and
(4) a process of making a plasma display apparatus, comprising the steps of providing dielectric substrates; forming a plurality of first electrodes on one of said substrates to extend in one direction; forming a plurality of second electrodes on the other substrate to extend in another direction perpendicular to said one direction; forming a ridge on at least one of said substrates to define a plurality of pixel areas; and providing fluorescent materials in said pixel areas, wherein the ridge is fabricated by a positive-acting diffusion patterning process comprising the sequential steps:
   a. Applying to at least one of the substrate an unpatterned first layer comprising a solid organic polymer which is soluble in a predetermined solvent or water;
   b. Applying to the unpatterned first layer a patterned second layer comprising a desolubilizing agent which is capable of decreasing the solubility of the organic polymer in the predetermined solvent or water;
   c. Heating the patterned second layer to effect patterned diffusion of the desolubilizing agent into the underlying first organic polymer layer to render the diffusion patterned areas of the polymer in the first layer insoluble in the predetermined solvent or water;
   d. Repeating the series of steps (a) to (c);
   e. Co-developing the non-patterned areas of the underlying first layer by washing with predetermined solvent or water; and
   f. Firing the patterned dielectric ridges.

In the process of the present invention, the diffusion pattering is used on layers of small thickness such as those used in the fabrication of electronic components. Typically the patterned layer of dielectric will range from 10 to 30 µm while the unpatterned layer of dielectric can be of much greater thickness from 10 to 100 µm. The thickness of the patterned layer is limited chiefly by the method of application rather than by considerations of operability.

The amount of solubilizing agent in the patterned layer must be sufficient to provide a solubilizing amount by diffusion to the underlying layer. Thus, the patterned layer will contain at least 10% weight solubilizing agent and may contain as much as 90% weight depending upon the solubility relationships of the respective polymers.

Furthermore, in some instances, it may be desirable to add a plasticizer or other solubilizing agent to the underlying unpatterned layer in order to make the polymer more susceptible to the action of the solubilizing agent which is diffused from the patterned layer.

By and large, the individual steps for preparation of components for the plasma display apparatus of the invention are similar to those which are known by those skilled in the art of conventional thick film, green tape and polymer technology. Thus, the following procedures may not be new by themselves, but illustrate a preferred method for formulating and preparing the materials to be used in the invention.

The dielectric pastes for the formation of the unpatterned layer are typically printed twice with 200 mesh screens at 2.5-5.1 cm (1-2 inches) per second squeegee speed. The patterning pastes are printed over the dielectric at higher speeds, since only a small part of the screen is open mesh.

The conductor pastes for the formation of electrodes are printed with a 325 or 400 mesh screen, depending on the conductor thickness and resolution desired. Patterning pastes are likewise printed with a 325 or 400 mesh screen, to optimize the amount of plasticizer delivered to the underprint. Thinner screens and fewer prints are needed than with the dielectric, because of the thinner films typically used with conductors.

Any polymers known in the art can be used as the material for the preparation of the above pastes. Representative examples of those polymers include cellulosic polymers such as ethyl cellulose, polystyrene polyacrylates (including methacrylates), poly(vinyl acetate), poly(vinyl butyral), poly(vinyl chloride) or phenol-formaldehyde resins.

It will be recognized by those skilled in polymer technology that each polymer species is compatible with a large number of different types of plasticizers or nonvolatile solvents. As a result, the number of suitable polymer/solvent/non-solvent combinations is legion.

Following are examples of several commercially available plasticizers which are compatible with ethyl cellulose, a typical polymer used in the patterning paste: acid esters of abietic acid (methyl abietate), acetic acid esters (cumphenylacetate), adipic acid derivatives (e.g. benzyloctyl adipate), diisodecyl adipate, tridecyl adipate), azelaic acid esters such as diisooctyl azelate, diethylene glycol dibenzoate, triethylene glycol dibenzoate, citrates such as triethyl citrate, epoxy type plasticizers, polyvinyl methyl ethers, glycerol mono-, di-, and triacetates, ethylene glycol diacetate, polyethylene glycol 200 to 1000, phthalate esters (dimethyl to dibutyl), isophthalic acid esters (dimethyl, diisooctyl, di-2-ethylhexyl), mellitates such as trioctyl trimellitate and isooctylisodecyl trimellitate, isopropyl myristate, methyl and propyl oleates, isopropyl and isooctyl palmitates, chlorinated paraffin, phosphoric acid derivatives such as triethyl phosphate, tributyl phosphate, tributoxyethyl phosphate, triphenyl phosphate, polyesters, dibutyl sebacate, dioctyl sebacate, stearates such as octyl stearate, butoxyethyl stearate, tetramethylene glycol monostearate, sucrose derivatives such as sucrose octoacetate, sulfonic acid derivatives such as benzenesulfonmethylamide, or dioctyl terephthalate.

Solvent/non-solvent systems for the ethyl cellulose/plasticizer combinations include:
Solvents: (D.S. denotes degree of substitution with ethoxyl groups.) D.S.=1.0 to 1.5: Pyridine, formic acid, acetic acid, water (cold) D.S.=2 Methylene chloride, chloroform, dichloroethylene, chlorohydrins, ethanol, THF. D.S.=2.3 Benzene, toluene, alkyl halogenides, alcohols, furan derivatives, ketones, acetic esters, carbon disulfide, nitromethane. D.S.=3.0 Benzene, toluene, methylene chloride, alcohols, esters.
Non-Solvents: D.S.=1.0 to 1.5: Ethanol. D.S.=2.0 Hydrocarbons, carbon tetrachloride, trichloroethylene, alcohols, diethyl ether, ketones, esters, water. D.S.=2.3 Ethylene glycol, acetate (cold). D.S.=3.0 Hydrocarbons, decalin, xylene, carbon tetrachloride, tetrahydrofurfuryl alcohol, diols, n-propyl ether.

### BRIEF DESCRIPTION OF THE DRAWINGS

Fig. 1 is an elevational view in section of the primary parts of a plasma display apparatus constructed in accordance with the present invention.

Fig. 2 is a foreshortened view in plan, partly in section of the plasma display apparatus.

Fig. 3 is a perspective view showing the structures of ridges and Y electrodes.

Fig. 4 and 5 are a series of views illustrating a sequence of steps in the process of the present invention.

Fig. 6 through 9 are a series of views illustrating another sequence of steps in the process of the present invention.

Fig. 10 is an elevational view in section of a plasma display apparatus constructed in accordance with the prior art.

### DETAILED DESCRIPTION OF THE INVENTION

Referring first to Figs. 1 and 2, there is shown a plasma display apparatus of the present invention which comprises first and second dielectric substrates 1, 2 of a sheet glass having a thickness equal to 2 mm, a plurality of X electrodes (first electrodes) laterally extending on the inner face of the first substrate 2, a plurality of Y electrodes (second electrodes) longitudinally extending on the inner face of the second substrate 2, and a plurality of fluorescent materials 5 for converting discharged ultraviolet rays into visible rays. The plasma display apparatus also comprises a matrix-like (or mesh-like) ridge 10 which defines a plurality of pixel areas and is adapted to provide a partition wall for maintaining the spacing between the first and second substrates 1, 2. Each of the (line) X electrodes 3 is disposed on dielectric layer 14 to electrically insulate from the (column) Y electrodes, and another dielectic layer 18 is arranged over the line electrodes 3 to separate from a discharge space 19. Protective layer 16 may be provided on dielectric layer 18. Each of the fluorescent materials 5 is formed by pouring a luminescence color fluorescent material into each of recesses 13 which are formed by the matrix-like ridge 10. The flurescent material may be Zn₂SiO₄:Mn for green color, (Y₁ Gd) BO₃:Eu³⁺ for red color or BaMgAl₁₄O₂₃:Eu²⁺ for blue color.

A discharge space 19 formed between the substrates 1, 2 by the matrix-like ridge 10 is filled with any suitable mixture gas, for example, consisting of neon and xenon. A discharge cell is formed at each of the intersections between the X electrodes 3 and the Y electrodes 4. When each discharging cell is energized, one fluorescent material 5 corresponding to the energized cell is excited to emit light.

In such an arrangement, the fluorescent material 5 may be selectively excited through the intersecting electrodes 3 and 4. As to the plasma display apparatus of the invention, any structural members mentioned from now are referred to Figs. 1-3.

The ridge in the plasma display apparatus may be produced in accordance with a negative acting pattern forming process shown in Figs. 4 and 5. The plasma display apparatus is fabricated with a ridge or a partition wall structure which is negatively patterned and sequentially developed as shown in Fig. 4 or negatively patterned and co-developed (as illustrated in Fig. 5) using diffusion patterning.

As illustrated in Fig. 4, a layer of thick film dielectric paste 23 is applied by screen printing to glass substrate 21. The thick film paste is comprised of finely divided particles of glass dispersed in an organic medium comprising an acid labile polymer dissolved in dibutyl phthalate plasticizer and terpineol. After printing the layer 23, the terpineol is removed by heating the layer to a temperature of 80°C for a period of 10 minutes.

A patterned second layer 25 is screen printed over the solvent-free thick film layer 23, the second layer is a liquid solution comprised of p-toluene sulfonic acid, dibutyl phthalate and terpineol, as shown in Fig. 4(b).

Upon forming the patterned layer 25, the assemblage is heated to 90°C during which the terpineol is evaporated from the layer and the acid and dibutyl phthalate are diffused into the underlying areas of thick film dielectric layer 23 whereby the acid reacts with the acid labile groups of the polymer to render it water dispersible (Fig. 4(c)).

The patterned layer 25 consists mainly of small amounts of residual acid and dibutyl phthalate. It is then washed with water having a pH of at least 7 to remove the underlying diffusion patterned layer 25, which consists largely of the solubilized acid labile polymer and the other materials in the underlying imaged areas of thick film layer 23. Upon completion of the washing, the surface of substrate 21 is exposed in the areas which underlay the pattern of layer 25 and a very precise negative image of the pattern remains on the surface of substrate 21 (Fig. 4(d)). The thus patterned dielectric is subsequently fired.

In such a manner, a matrix-like ridge 10 is formed by the layer such that a discharge space for each pixel area is formed by each of the recesses 13 having, for example, a depth ranged between 25 and 100 µm depending on the pitch size of pixel. When it is desirable to obtain a thicker or more raised ridge, one may repeat a series of the steps of dielectric print/dry through development as shown in Figs. 4-8. Fig. 5 illustrates schematically the process of producing the same negatively patterned and co-developed by use of 2 or 3 diffusion patterning steps.

After desirable thickness of the ridge is obtained, the dielectric is fired on the surface of the glass substrate 21, conductor is applied to form the line and column of electrodes on the other glass substrate 2 opposing the substrate 21 as described previously. Each group of the electrodes is formed by the screen printing process (thick film process) wherein a paste containing a metal selected from the group consisting of Au, Ni, Al, Cu and silver as a principal component is applied and then fired to form an electrode layer which is used to form each group of electrodes. The material of this electrode layer is then partially removed to form the electrodes. Thus, the width of the electrode layer may be larger than that of the final electrode.

By the use of the screen printing process, the overall surface of the glass substrate 2 is coated with a lead borate, low melting glass paste containing a dielectric material such as aluminum oxide or silicon oxide. The paste is then fired to form dielectric layers 14 and 18. The glass substrate 2 may include a protective layer 16 of magnesium oxide which is formed over the dielectric layer.

Each of the recesses 13 defined by the ridge 10 is filled with a fluorescent material 5 at the bottom.

When to be used for monocolor display, each of the fluorescent material 5 is formed by depositing a fluorescent material on the inner bottom face 13 of the corresponding recess, for example, Zn₂SiO₄ emitting a green-colored light. If it is wanted to provide a multicolor display, fluorescent materials for emitting red(R)-, green(G)- and blue(B)-colors are sequentially deposited on the inner bottom face of each discharge area for each pixel area line in the X or Y direction or for each pixel area PA (Fig. 3).

When it is desirable, the said diffusion patterning process may be applied to both substrates 1 and 2 to fabricate the ridge or the entire partition wall.

Thereafter, the glass substrate 2 is superposed over the display side glass substrate 1. The space between the glass substrates 1, 2 is sealed by sealing glass and at the same time a discharge mixture gas is sealingly enclosed in the space. A plasma display apparatus is thus assembled.

Referring further to Figs. 6 and 7, an alternative process of fabricating a ridge or partition wall in the plasma display apparatus of the invention is explained, for instance, a positive-acting non-photographic method for making patterns in dielectric films comprising the sequential steps:
a. Applying to a substrate 111 an unpatterned first layer 113 comprising a solid organic polymer which is soluble in a predetermined solvent or water;
b. Applying to the unpatterned first layer 113 a patterned second layer 115 comprising a desolubilizing agent which is capable of decreasing the solubility of the organic polymer in the solvent;
c. Heating the patterned second layer 115 to effect patterned diffusion of the desolubilizing agent into the underlying first organic polyer layer 113 and to render the diffusion patterned areas of the polymer in the first layer 113 insoluble in the solvent; and
d. Removing the non-patterned areas of the underlying first layer 113 by washing them in the predetermined solvent.

If the insolubilizer-depleted areas of the patterned second layer 115 are soluble in the solvent, they will be removed during the solvent-washing step (Fig. 6 (a) to (d)). On the other hand, if the insolubilizer-depleted areas of the patterned second layer 115 are insoluble-in the solvent, they will remain after the solvent-washing step ( Fig. 7 (a) to (d)).

After removal of the solvent, the unpatterned layer 113 comprising an organic polymer or the patterned layer 115 comprising a polymer insoluble in the solvent and the corresponding organic polymer layer 113 are left on the substrate to form a matrix-like ridge 10 defining pixel areas in the plasma display and forming a discharge space. The remaining steps for producing the plasma display are similar to those of the aforementioned process.

A plurality of positive-acting diffusion patterning steps are used to build up partition wall thickness. Figs. 6 and 7 illustrate schematically the steps involved to apply up to 3 DP steps.

Alternatively, one may also reduce the number of developing step by using the process illustrated in Figs. 8 and 9. Fig. 8 represents the case that the DP layers are insoluble in the developing solvent. If the DP layer became soluble after being depleted of the insolubilizing agent, only top of the built became insoluble since the lower DP layers remain insoluble after receiving supply of desolubilizing agent from the DP layer immediately above the said layer. This is illustrated in Fig. 9 (f) to (i).

The above method can also be applied to both substrates 1 and 2, if desirable.

Although some embodiments of the present invention have been described as to ridges 10 usable as partition walls for parting display pixels, the partition walls are formed on the display side of glass substrates 2 separately of the ridge 10 formed on the first substrate 1.

The following example illustrates the formulation of dielectric and patterning pastes.

### Example 1

Two pastes were formulated: One a dielectric paste, and one a patterning paste as follows:

| Dielectric Paste | |
|---|---|
| Glass A | 15.78 grams |
| Glass B | 0.83 |
| Alumina A | 7.89 |
| Alumina B | 3.24 |
| Cobalt Aluminate | 0.08 |
| Polymethyl methacrylate | 5.36 |
| Wetting Agent | 1.25 |
| t-Butylanthraquinone | 0.50 |
| Shell Ionol® | 0.03 |
| Butyl Carbitol®, Acetate | 14.10 |
| Butyl Benzyl Phthalate | 0.75 |

| Glass A | |
|---|---|
| SiO₂ | 56.2% wt. |
| PbO | 18.0 |
| Al₂O₃ | 8.6 |
| CaO | 7.4 |
| B₂O₃ | 4.5 |
| Na₂O | 2.7 |
| K₂O | 1.6 |
| MgO | 0.8 |
| ZrO₂ | 0.2 |

Glass A has a D₅₀ of ca. 4 to 4.5 µm; it is milled and classified to remove coarse and fine fractions. Its D₁₀ is about 1.6 microns; and D₉₀ is 10-12 microns. Surface area is 1.5 to 1.8 m²/g.

Glass B is a barium borosilicate glass used to lower the sintering temperature of the dielectric composite, due to the large particle size of glass A. Its formula follows:

| | |
|---|---|
| BaO | 37.5% wt. |
| B₂O₃ | 38.3 |
| SiO₂ | 16.5 |
| MgO | 4.3 |
| ZrO₂ | 3.0 |

Alumina A is a 1 micron powder with a narrow particle size distribution: D₁₀, D₅₀, and D₉₀ are, respectively, ca. 0.5, 1.1, and 2.7 microns. It is classified by settling to remove coarses and fines. Surface area is about 2.7-2.8 m²/g.

Alumina B is a 0.4 micron average particle size powder with surface area of about 5 m²/g.

| Patterning Paste | |
|---|---|
| Alumina A | 60.0 grams |
| Hydrogenated Castor Oil | 1.4 |
| Mineral Spirits | 4.0 |
| Colorant | 2.2 |
| Ethyl Cellulose T-200 | 4.3 |
| Terpineol | 11.9 |
| Butyl Benzyl Phthalate | 16.2 |

The above paste compositions were prepared in the manner familiar to those skilled in formulation of thick film materials and were prepared for printing as follows:

The materials were processed by printing the dielectric optionally one, two, or three prints, with each print followed by drying 10 to 15 minutes at 80 to 90 °C. The patterning layer was then printed by using a via fill screen with several sizes of via openings. The patterning paste was then dried at 80 to 100 °C for 5 to 10 minutes.

The pattern was then generated in the dielectric by immersing the overpinted layers in 1.1.1-trichloroethane with ultrasonic agitation until the overprinted areas were removed and the areas under the overprinted patterning paste were dissolved away.

Vias as small as 127-178 µm (5-7 mils) were resolved in dielectric films as thick as 85 µm with good edge definition. This is far superior both in resolution and in thickness achievable with a single patterning step with screen printing.

### Alternative Material Systems

There are many ways to use the selective solubilization principle to generate thick film patterns. The pattern may be positive or negative working, i.e. the area under the overprint may either be solubilized, as in Examples 2-3 or it may be insolubilized, for example by overprinting an aqueously developable polymer with a water incompatible plasticizer to protect the areas underneath, then removing the unplasticized material by aqueous solubilization.

The following Table illustrates a number of acrylic polymer/plasticizer/solvent systems which have been demonstrated for use in the method of the invention.

| Alternative Acrylic Material Systems | | | |
|---|---|---|---|
| Underprint Resin | Overprint | | Patterning Solvent |
| | Solubilizer (Negative) | Desolubilizer (Positive) | |
| Polymethylmethacrylate Phthalate | Methyl Chloroform | | Dibutyl |
| Polymethylacrylate | Butyl Benzyl-Phthalate | | |
| | Ethylhydroxyethyl cellulose | | |
| | | Polymethyl methacrylate | Ethanol/water/ammonia |
| Carboset® XPD-1234 | Triethanolamine | | Water |
| | | Dibutyl phthalate | K₂CO₃/Water |

The above resins may be combined. For example, methyl and ethyl methacrylate may be combined to allow positive or negative working resists. In the case of methyl methacrylate/ethyl methacrylate combinations, plasticizers such as triethylene glycol would produce a negative working resist in ethanol pattern generating solvent.

The following examples illustrate the paste formulation which have been demonstrated for use in the method for fabricating the plasma display according to the invention.

### Examples 2 and 3

### Aqueous Diffusion Patterning

A calcium zinc silicate glass was formulated with a cellulosic vehicle and 3% butyl benzyl phthalate. A film of each paste was screen printed onto an alumina substrate and dried at 95°-100°C. A patterning paste containing 7 g alumina, 3.5 g Tergitol® TMN-6, 3.15 g of terpineol isomers and 0.35 g ethyl cellulose was screen printed onto the dried dielectric paste layers and heated at 95°-100°C to dry the overprinted paste and to effect diffusion of the Tergitol detergent into the underlying dielectric layer. When the dried layer was washed under tap water, 152 µm (6mil) vias were clearly resolved. In subsequent tests, it was shown that the use of additional plasticizer in the underlying polymer layer improved resolution still further.

It is preferred to carry out the diffusion patterning process to fabricate a partition wall in the plasma display apparatus as described in Examples 2-3. Nevertheless, it can be carried out by other methods, for example by overprinting an aqueous developable polymer with a water incompatible plasticizer to protect the areas underneath, then removing the unplasticized material by aqueous solubilization.

## Claims

1. A process of making a plasma display apparatus, comprising the steps of providing dielectric substrates; forming a plurality of first electrodes on one of said substrates to extend in one direction; forming a plurality of second electrodes on the other substrate to extend in another direction perpendicular to said one direction; forming a ridge on at least one of said substrates to define a plurality of pixel areas; and providing fluorescent materials in said pixel areas, wherein the ridge is fabricated by a negative-acting diffusion patterning process comprising the sequential steps:
a. Applying to at least one of the substrate an unpatterned first layer comprising a solid organic polymer which is soluble in a predetermined solvent or water;
b. Applying to the unpatterned first layer a patterned second layer comprising a solubilizing agent which is capable of increasing the solubility of the organic polymer in the predetermined solvent or water;
c. Heating the patterned second layer to effect patterned diffusion of the solubilizing agent into the underlying first organic polymer layer to render the diffusion patterned areas of the polymer in the first layer soluble in the predetermined solvent or water;
d. Developing the underlying patterned layers by washing with predetermined solvent or water;
e. Repeating a series of the above steps (a) to (d) to build thicker or more raised ridges; and
f. Firing the patterned dielectric ridges.

2. A process of making a plasma display apparatus, comprising the steps of providing dielectric substrates; forming a plurality of first electrodes on one of said substrates to extend in one direction; forming a plurality of second electrodes on the other substrate to extend in another direction perpendicular to said one direction; forming a ridge on at least one of said substrates to define a plurality of pixel areas; and providing fluorescent materials in said pixel areas, wherein the ridge is fabricated by a negative-acting diffusion patterning process comprising the sequential steps:
a. Applying to at least one of the substrate an unpatterned first layer comprising a solid organic polymer which is soluble in a predetermined solvent or water;
b. Applying to the unpatterned first layer a patterned second layer comprising a solubilizing agent which is capable of increasing the solubility of the organic polymer in the predetermined solvent or water;
c. Heating the patterned second layer to effect patterned diffusion of the solubilizing agent into the underlying first organic polymer layer to render the diffusion patterned areas of the polymer in the first layer soluble in the predetermined solvent or water;
d. Repeating the series of steps (a) to (c);
e. Co-developing the underlying patterned layers by washing with predetermined solvent or water; and
f. Firing the patterned dielectric ridges.

3. A process of making a plasma display apparatus, comprising the steps of providing dielectric substrates; forming a plurality of first electrodes on one of said substrates to extend in one direction; forming a plurality of second electrodes on the other substrate to extend in another direction perpendicular to said one direction; forming a ridge on at least one of said substrates to define a plurality of pixel areas; and providing fluorescent materials in said pixel areas, wherein the ridge is fabricated by a positive-acting diffusion patterning process comprising the sequential steps:
a. Applying to at least one of the substrate an unpatterned first layer comprising a solid organic polymer which is soluble in a predetermined solvent or water;
b. Applying to the unpatterned first layer a patterned second layer comprising a desolubilizing agent which is capable of decreasing the solubility of the organic polymer in the predetermined solvent or water;
c. Heating the patterned second layer to effect patterned diffusion of the desolubilizing agent into the underlying first organic polymer layer to render the diffusion patterned areas of the polymer in the first layer insoluble in the predetermined solvent or water;
d. Developing the non-patterned areas of the underlying first layer by washing with predetermined solvent water;
e. Repeating a series of the above steps (a) to (d) to build thicker or more raised ridges; and
f. Firing the patterned dielectric ridges.

4. A process of making a plasma display apparatus, comprising the steps of providing dielectric substrates; forming a plurality of first electrodes on one of said substrates to extend in one direction; forming a plurality of second electrodes on the other substrate to extend in another direction perpendicular to said one direction; forming a ridge on at least one of said substrates to define a plurality of pixel areas; and providing fluorescent materials in said pixel areas, wherein the ridge is fabricated by a positive-acting diffusion patterning process comprising the sequential steps:
a. Applying to at least one of the substrate an unpatterned first layer comprising a solid organic polymer which is soluble in a predetermined solvent or water;
b. Applying to the unpatterned first layer a patterned second layer comprising a desolubilizing agent which is capable of decreasing the solubility of the organic polymer in the predetermined solvent or water;
c. Heating the patterned second layer to effect patterned diffusion of the desolubilizing agent into the underlying first organic polymer layer to render the diffusion patterned areas of the polymer in the first layer insoluble in the predetermined solvent or water;
d. Repeating the series of steps (a) to (c);
e. Co-developing the non-patterned areas of the underlying first layer by washing with predetermined solvent or water; and
f. Firing the patterned dielectric ridges.

## Patentansprüche

1. Verfahren zur Herstellung eines Plasmaanzeigegeräts, umfassend die Stufen der Bereitstellung dielektrischer Substrate; der Bildung einer Mehrzahl erster Elektroden auf einem der Substrate, so daß sie sich in einer Richtung erstrecken; der Bildung einer Mehrzahl zweiter Elektroden auf dem anderen Substrat, so daß sie sich in einer anderen Richtung erstrecken, die senkrecht zu der einen Richtung steht; der Bildung eines Stegs auf wenigstens einem der Substrate, um eine Mehrzahl von Pixel-bereichen zu definieren; und der Bereitstellung von fluoreszierenden Materialien in den Pixelbereichen, worin der Steg durch ein negativ-wirkendes, musterbildendes Diffusionsverfahren hergestellt wird, umfassend die aufeinanderfolgenden Stufen:
a. des Auftragens einer ungemusterten ersten Schicht, umfassend ein festes, organisches Polymer, das in einem vorherbestimmten Lösungsmittel oder Wasser löslich ist, auf wenigstens eines der Substrate;
b. des Auftragens einer gemusterten zweiten Schicht, umfassend ein Solubilisierungsmittel, das die Löslichkeit des organischen Polymers in dem vorherbestimmten Lösungsmittel oder Wasser erhöhen kann, auf die ungemusterte erste Schicht;
c. des Erwärmens der gemusterten zweiten Schicht, um eine musterbildende Diffusion des Solubilisierungsmittels in die darunterliegende erste organische Polymerschicht zu bewirken, um die durch Diffusion gemusterten Bereiche des Polymers in der ersten Schicht in dem vorherbestimmten Lösungsmittel oder Wasser löslich zu machen;
d. des Entwickelns der darunterliegenden gemusterten Schichten durch Waschen mit dem vorherbestimmten Lösungsmittel oder Wasser;
e. des Wiederholens einer Reihe der obigen Stufen (a) bis (d), um dickere oder erhöhtere Stege herzustellen; und
f. des Brennens der gemusterten dielektrischen Stege.

2. Verfahren zur Herstellung eines Plasmaanzeigegeräts, umfassend die Stufen der Bereitstellung dielektrischer Substrate; der Bildung einer Mehrzahl erster Elektroden auf einem der Substrate, so daß sie sich in einer Richtung erstrecken; der Bildung einer Mehrzahl zweiter Elektroden auf dem anderen Substrat, so daß sie sich in einer anderen Richtung erstrecken, die senkrecht zu der einen Richtung steht; der Bildung eines Stegs auf wenigstens einem der Substrate, um eine Mehrzahl von Pixel-bereichen zu definieren; und der Bereitstellung von fluoreszierenden Materialien in den Pixelbereichen, worin der Steg durch ein negativ-wirkendes, musterbildendes Diffusionsverfahren hergestellt wird, umfassend die aufeinanderfolgenden Stufen:
a. des Auftragens einer ungemusterten ersten Schicht, umfassend ein festes, organisches Polymer, das in einem vorherbestimmten Lösungsmittel oder Wasser löslich ist, auf wenigstens eines der Substrate;
b. des Auftragens einer gemusterten zweiten Schicht, umfassend ein Solubilisierungsmittel, das die Löslichkeit des organischen Polymers in dem vorherbestimmten Lösungsmittel oder Wasser erhöhen kann, auf die ungemusterte erste Schicht;
c. des Erwärmens der gemusterten zweiten Schicht, um eine musterbildende Diffusion des Solubilisierungsmittels in die darunterliegende erste organische Polymerschicht zu bewirken, um die durch Diffusion gemusterten Bereiche des Polymers in der ersten Schicht in dem vorherbestimmten Lösungsmittel oder Wasser löslich zu machen;
d. des Wiederholens der Reihe der Stufen (a) bis (c);
e. des gemeinsamen Entwickelns der darunterliegenden gemusterten Schichten durch Waschen mit dem vorherbestimmten Lösungsmittel oder Wasser; und
f. des Brennens der gemusterten dielektrischen Stege.

3. Verfahren zur Herstellung eines Plasmaanzeigegeräts, umfassend die Stufen der Bereitstellung dielektrischer Substrate; der Bildung einer Mehrzahl erster Elektroden auf einem der Substrate, so daß sie sich in einer Richtung erstrecken; der Bildung einer Mehrzahl zweiter Elektroden auf dem anderen Substrat, so daß sie sich in einer anderen Richtung erstrecken, die senkrecht zu der einen Richtung steht; der Bildung eines Stegs auf wenigstens einem der Substrate, um eine Mehrzahl von Pixelbereichen zu definieren; und der Bereitstellung von fluoreszierenden Materialien in den Pixelbereichen, worin der Steg durch ein positiv-wirkendes, musterbildendes Diffusionsverfahren hergestellt wird, umfassend die aufeinanderfolgenden Stufen:
a. des Auftragens einer ungemusterten ersten Schicht, umfassend ein festes, organisches Polymer, das in einem vorherbestimmten Lösungsmittel oder Wasser löslich ist, auf wenigstens eines der Substrate;
b. des Auftragens einer gemusterten zweiten Schicht, umfassend ein Desolubilisierungsmittel, das die Löslichkeit des organischen Polymers in dem vorherbestimmten Lösungsmittel oder Wasser verringern kann, auf die ungemusterte erste Schicht;
c. des Erwärmens der gemusterten zweiten Schicht, um eine musterbildende Diffusion des Desolubilisierungsmittels in die darunterliegende erste organische Polymerschicht zu bewirken, um die durch Diffusion gemusterten Bereiche des Polymers in der ersten Schicht in dem vorherbestimmten Lösungsmittel oder Wasser unlöslich zu machen;
d. des Entwickelns der ungemusterten Bereiche der darunterliegenden ersten Schicht durch Waschen mit dem vorherbestimmten Lösungsmittel oder Wasser;
e. des Wiederholens einer Reihe der obigen Stufen (a) bis (d), um dickere oder erhöhtere Stege herzustellen; und
f. des Brennens der gemusterten dielektrischen Stege.

4. Verfahren zur Herstellung eines Plasmaanzeigegeräts, umfassend die Stufen der Bereitstellung dielektrischer Substrate; der Bildung einer Mehrzahl erster Elektroden auf einem der Substrate, so daß sie sich in einer Richtung erstrecken; der Bildung einer Mehrzahl zweiter Elektroden auf dem anderen Substrat, so daß sie sich in einer anderen Richtung erstrecken, die senkrecht zu der einen Richtung steht; der Bildung eines Stegs auf wenigstens einem der Substrate, um eine Mehrzahl von Pixelbereichen zu definieren; und der Bereitstellung von fluoreszierenden Materialien in den Pixelbereichen, worin der Steg durch ein positiv-wirkendes, musterbildendes Diffusionsverfahren hergestellt wird, umfassend die aufeinanderfolgenden Stufen:
a. des Auftragens einer ungemusterten ersten Schicht, umfassend ein festes, organisches Polymer, das in einem vorherbestimmten Lösungsmittel oder Wasser löslich ist, auf wenigstens eines der Substrate;
b. des Auftragens einer gemusterten zweiten Schicht, umfassend ein Desolubilisierungsmittel, das die Löslichkeit des organischen Polymers in dem vorherbestimmten Lösungsmittel oder Wasser verringern kann, auf die ungemusterte erste Schicht;
c. des Erwärmens der gemusterten zweiten Schicht, um eine musterbildende Diffusion des Desolubilisierungsmittels in die darunterliegende erste organische Polymerschicht zu bewirken, um die durch Diffusion gemusterten Bereiche des Polymers in der ersten Schicht in dem vorherbestimmten Lösungsmittel oder Wasser unlöslich zu machen;
d. des Wiederholens der Reihe der Stufen (a) bis (c);
e. des gemeinsamen Entwickelns der ungemusterten Bereiche der darunterliegenden ersten Schicht durch Waschen mit dem vorherbestimmten Lösungsmittel oder Wasser; und
f. des Brennens der gemusterten dielektrischen Stege.

## Revendications

1. Procédé de fabrication d'un appareil d'affichage à plasma, comprenant les étapes de fourniture de substrats diélectriques; de formation sur l'un desdits substrats d'une pluralité de premières électrodes s'étendant dans une direction; de formation sur l'autre substrat d'une pluralité de deuxièmes électrodes s'étendant dans l'autre direction perpendiculaire à ladite première direction; de formation d'une arête sur au moins un desdits substrats afin de définir une pluralité d'aires de pixel, et de fourniture de matériaux fluorescents dans lesdites aires de pixel, dans lequel l'arête est obtenue par un procédé de formation des motifs par diffusion à action négative comprenant les étapes séquentielles suivantes :
a. application sur au moins un des substrats d'une première couche sans motif contenant un polymère organique solide soluble dans un solvant prédéterminé ou dans l'eau;
b. application sur la première couche sans motif d'une deuxième couche à motifs contenant un agent de solubilisation capable d'augmenter la solubilité du polymère organique dans le solvant prédéterminé ou dans l'eau;
c. cuisson de la deuxième couche à motifs pour effectuer la diffusion suivant des motifs de l'agent de solubilisation dans la première couche de polymère organique sous-jacente pour rendre les zones du polymère, où les motifs ont été formés par diffusion dans la première couche, solubles dans le solvant prédéterminé ou dans l'eau;
d. développement des couches sous-jacentes à motifs en lavant avec le solvant prédéterminé ou l'eau;
e. répétition d'une succession d'étapes (a) à (d) mentionnées plus haut pour former des arêtes plus épaisses ou plus élevées, et
f. cuisson des arêtes à motifs diélectriques.

2. Procédé de fabrication d'un appareil d'affichage à plasma, comprenant les étapes de fourniture de substrats diélectriques; de formation sur l'un desdits substrats d'une pluralité de premières électrodes s'étendant dans une direction; de formation sur l'autre substrat d'une pluralité de deuxièmes électrodes s'étendant dans l'autre direction perpendiculaire à la première direction; de formation d'une arête sur au moins un desdits substrats afin de définir une pluralité d'aires de pixel, et de fourniture de matériaux fluorescents dans lesdites aires de pixel, dans lequel l'arête est obtenue par un procédé de formation des motifs par diffusion à action négative comprenant les étapes séquentielles suivantes :
a. application sur au moins un des substrats d'une première couche sans motif contenant un polymère organique solide soluble dans un solvant prédéterminé ou dans l'eau;
b. application sur la première couche sans motif d'une deuxième couche à motifs contenant un agent de solubilisation capable d'augmenter la solubilité du polymère organique dans le solvant prédéterminé ou dans l'eau;
c. cuisson de la deuxième couche à motifs pour effectuer la diffusion suivant des motifs de l'agent de solubilisation dans la première couche de polymère organique pour rendre les zones du polymère, où les motifs ont été formés par diffusion dans la première couche, solubles dans le solvant prédéterminé ou dans l'eau;
d.- répétition de la succession d'étapes (a) à (c);
e. co-développement des couches sous-jacentes à motifs en lavant avec le solvant prédéterminé ou de l'eau, et
f. cuisson des arêtes à motifs diélectriques.

3. Procédé de fabrication d'un appareil d'affichage à plasma, comprenant les étapes de fourniture de substrats diélectriques; de formation sur l'un desdits substrats d'une pluralité de premières électrodes s'étendant dans une direction; de formation sur l'autre substrat d'une pluralité de deuxièmes électrodes s'étendant dans l'autre direction perpendiculaire à la première direction; de formation d'une arête sur au moins un desdits substrats afin de définir une pluralité d'aires de pixel, et de fourniture de matériaux fluorescents dans lesdites aires de pixel, dans lequel l'arête est obtenue par un procédé de formation des motifs par diffusion à action positive comprenant les étapes séquentielles suivantes :
a. application sur au moins un des substrats d'une première couche sans motif contenant un polymère organique solide soluble dans un solvant prédéterminé ou dans l'eau;
b. application sur la première couche sans motif d'une deuxième couche à motifs contenant un agent de désolubilisation capable de diminuer la solubilité du polymère organique dans le solvant prédéterminé ou dans l'eau;
c. cuisson de la deuxième couche à motifs pour effectuer la diffusion suivant des motifs de l'agent de désolubilisation sur la première couche de polymère organique sous-jacente pour rendre les zones du polymère, où les motifs ont été formés par diffusion dans la première couche, insolubles dans le solvant prédéterminé ou dans l'eau;
d. développement des couches sans motif de la première couche sous-jacente en lavant avec le solvant prédéterminé ou de l'eau;
e. répétition d'une succession d'étapes (a) à (d) mentionnées plus haut pour former des arêtes plus épaisses ou plus élevées, et
f. cuisson des arêtes à motifs diélectriques.

4. Procédé de fabrication d'un appareil d'affichage à plasma, comprenant les étapes de fourniture de substrats diélectriques; de formation sur l'un desdits substrats d'une pluralité de premières électrodes s'étendant dans une direction; de formation sur l'autre substrat d'une pluralité de deuxièmes électrodes s'étendant dans l'autre direction perpendiculaire à la première direction; de formation d'une arête sur au moins un desdits substrats afin de définir une pluralité d'aires de pixel, et de fourniture de matériaux fluorescents dans lesdites aires de pixel, dans lequel l'arête est obtenue par un procédé de formation des motifs par diffusion à action positive comprenant les étapes séquentielles suivantes :
a. application sur au moins un des substrats d'une première couche sans motif contenant un polymère organique solide soluble dans un solvant prédéterminé ou dans l'eau;
b. application sur la première couche sans motif d'une deuxième couche à motifs contenant un agent de désolubilisation capable de diminuer la solubilité du polymère organique dans le solvant prédéterminé ou dans l'eau;
c. cuisson de la deuxième couche à motifs pour effectuer la diffusion suivant des motifs de l'agent de désolubilisation dans la première couche de polymère organique sous-jacente pour rendre les zones du polymère, où les motifs ont été formés par diffusion dans la première couche, insolubles dans le solvant prédéterminé ou dans l'eau;
d.- répétition de la succession d'étapes (a) à (c);
e. co-développement des couches sans motif de la première couche sous-jacente en lavant avec le solvant prédéterminé ou de l'eau, et f. cuisson des arêtes à motifs diélectriques.
